



US008137880B2

(12) **United States Patent**  
**Wosnick et al.**

(10) **Patent No.:** **US 8,137,880 B2**  
(45) **Date of Patent:** **Mar. 20, 2012**

(54) **COLORED TONERS**

(75) Inventors: **Jordan H. Wosnick**, Toronto (CA);  
**Richard P. N. Veregin**, Mississauga (CA); **Eric Rotberg**, Toronto (CA)

(73) Assignee: **Xerox Corporation**, Norwalk, CT (US)

(\*) Notice: Subject to any disclaimer, the term of this patent is extended or adjusted under 35 U.S.C. 154(b) by 0 days.

(21) Appl. No.: **12/690,360**

(22) Filed: **Jan. 20, 2010**

(65) **Prior Publication Data**

US 2011/0177443 A1 Jul. 21, 2011

(51) **Int. Cl.**

**G03G 9/09** (2006.01)

(52) **U.S. Cl.** ..... **430/108.1**; 430/108.2; 430/108.21; 430/108.24; 430/109.1; 430/109.4

(58) **Field of Classification Search** ..... 430/108.1, 430/109.1, 109.4, 108.2, 108.21, 108.24

See application file for complete search history.

(56) **References Cited**

## U.S. PATENT DOCUMENTS

|             |         |                  |
|-------------|---------|------------------|
| 3,590,000 A | 6/1971  | Palermi et al.   |
| 3,655,374 A | 4/1972  | Palermi et al.   |
| 3,720,617 A | 3/1973  | Chatterji et al. |
| 3,847,604 A | 11/1974 | Hagenbach et al. |
| 3,944,493 A | 3/1976  | Jadwin et al.    |
| 3,983,045 A | 9/1976  | Jugle et al.     |
| 4,007,293 A | 2/1977  | Mincer et al.    |

|                   |          |                                 |
|-------------------|----------|---------------------------------|
| 4,079,014 A       | 3/1978   | Burness et al.                  |
| 4,295,990 A       | 10/1981  | Verbeek et al.                  |
| 4,394,430 A       | 7/1983   | Jadwin et al.                   |
| 4,560,635 A       | 12/1985  | Hoffend et al.                  |
| 4,935,326 A       | 6/1990   | Creatura et al.                 |
| 4,937,166 A       | 6/1990   | Creatura et al.                 |
| 5,236,629 A       | 8/1993   | Mahabadi et al.                 |
| 5,290,654 A       | 3/1994   | Sacripante et al.               |
| 5,302,486 A       | 4/1994   | Patel et al.                    |
| 5,330,874 A       | 7/1994   | Mahabadi et al.                 |
| 5,723,245 A       | 3/1998   | Bertrand et al.                 |
| 5,734,800 A       | 3/1998   | Herbert et al.                  |
| 5,866,288 A       | * 2/1999 | Ciccarelli et al. .... 430/45.4 |
| 6,004,714 A       | 12/1999  | Ciccarelli et al.               |
| 6,063,827 A       | * 5/2000 | Sacripante et al. .... 522/6    |
| 6,066,421 A       | 5/2000   | Julien et al.                   |
| 6,190,815 B1      | 2/2001   | Ciccarelli et al.               |
| 6,593,049 B1      | 7/2003   | Veregin et al.                  |
| 6,756,176 B2      | 6/2004   | Stegamat et al.                 |
| 6,809,837 B1      | 10/2004  | Mestha et al.                   |
| 6,830,860 B2      | 12/2004  | Sacripante et al.               |
| 7,123,380 B2      | 10/2006  | Van de Capelle                  |
| 7,375,851 B2      | 5/2008   | Mestha                          |
| 2004/0063013 A1 * | 4/2004   | Hongo et al. .... 430/59.1      |
| 2005/0227160 A1 * | 10/2005  | Shirai et al. .... 430/109.4    |
| 2006/0222991 A1   | 10/2006  | Sacripante et al.               |
| 2009/0028614 A1   | 1/2009   | Kerkhali et al.                 |

\* cited by examiner

Primary Examiner — Peter Vajda

(74) Attorney, Agent, or Firm — MDIP LLC

(57) **ABSTRACT**

The present disclosure provides blue toners and methods for their production. In embodiments, methods of the present disclosure include systems which may be utilized to predict the color properties of a blue toner, thereby permitting adjustment of the pigment loading and/or toner mass per unit area.

17 Claims, 4 Drawing Sheets



**FIG. 1**



**FIG. 2**

**FIG. 3**



# 1

## COLORED TONERS

### BACKGROUND

The present disclosure provides an approach for producing colored toner compositions and, in embodiments, to a system and method for predicting color properties of toner compositions.

In today's business and scientific world, color has become essential as a component of communication. Color facilitates the sharing of knowledge and ideas. Companies involved in the development of digital color print engines are continuously looking for ways to improve the image quality of their products. One of the elements that affects image quality is the ability to consistently produce the same image on a printer from one day to another, from one week to the next, month after month. Users have become accustomed to printers and copiers that produce high quality color and gray-scaled output. Users now expect to be able to reproduce a color image with consistent quality on any compatible printing device, including another device within an organization, a device at home, or a device used anywhere else in the world.

Color images are commonly represented as one or more separations, each separation comprising a set of color density signals for a single primary or secondary color. Color density signals are commonly represented as digital gray or contone pixels, varying in magnitude from a minimum to a maximum, with a number of gradients corresponding to the bit density of the system. Thus, a common 8-bit system provides 256 shades of each primary color. A color can therefore be considered the combination of magnitudes of each pixel, which when viewed together, present the combination color.

CMYK is a color model in which all colors are described as a mixture of four process colors (i.e., cyan, magenta, yellow, and black). CMYK is the standard color model used in offset printing for full-color documents. Because such printing uses inks of these four basic colors, it is often called four-color printing and is a subtractive color model. The CMYK model works by partially or entirely masking certain colors on the typically white background (that is, absorbing particular wavelengths of light). Such a model is called subtractive because inks "subtract" brightness from white. In additive color models such as RGB (i.e., red, green, blue), white is the "additive" combination of all primary colored lights, while black is the absence of light. In the CMYK model, it is just the opposite. In other words, white is the natural color of the paper or other background, while black results from a full combination of colored inks. To save money on ink, and to produce deeper black tones, unsaturated and dark colors are produced by substituting black ink for the combination of cyan, magenta and yellow.

There are different ways of representing color. One way color is described consists of the following parameters: hue, lightness and saturation. Hue represents the actual color wavelength (red, blue, etc.); lightness corresponds to the white content; while saturation captures the richness or amplitude in color. Another way of describing color uses the three dominant primary colors: red, green, and blue (RGB). By combining these primary colors, in different intensities, most colors visible to humans can be reproduced.

While the CMYK color space is the standard color space used by production printers, the Red-Green-Blue (RGB) color space is a personal computer's native color space. As a result, display devices generally use a different color model, namely the RGB model. One of the most difficult aspects of desktop publishing in color is color matching, which is prop-

erly converting the RGB colors into CMYK colors so that what gets printed looks the same as what appears on the monitor.

One issue with the CMYK color space is that the standard CMYK color set on its own provides relatively poor representation of saturated blue hues.

Improved methods for producing colored toners, including systems that are not device-dependent, remain desirable.

10

### SUMMARY

The present disclosure provides colored toners and processes for producing same. In embodiments, the present disclosure provides a blue toner including at least one resin; an optional wax; and a colorant system including a violet pigment such as Pigment Violet 23, Pigment Violet 3, and combinations thereof, in combination with a cyan pigment such as Pigment Blue 61, Pigment Blue 15:3, Pigment Blue 15:4, Pigment Blue 1, Pigment Blue 15:1, Pigment Blue 15:2, and combinations thereof, wherein the blue toner matches the color of a blue selected from the group consisting of Pantone Blue 072 and Pantone Reflex Blue within a human perception limit ( $\Delta E_{2000}$ ) of less than about 3.

In other embodiments, a blue toner of the present disclosure includes at least one amorphous polyester resin in combination with at least one crystalline polyester resin; a wax; and a colorant system including a violet pigment such as Pigment Violet 23, Pigment Violet 3, and combinations thereof, in combination with a cyan pigment such as Pigment Blue 61, Pigment Blue 15:3, Pigment Blue 15:4, Pigment Blue 1, Pigment Blue 15:1, Pigment Blue 15:2, and combinations thereof, wherein the blue toner matches the color of a blue selected from the group consisting of Pantone Blue 072 and Pantone Reflex Blue within a human perception limit ( $\Delta E_{2000}$ ) of less than about 3.

A process of the present disclosure may include, in embodiments, contacting at least one resin and at least one surfactant to form an emulsion; contacting the emulsion with an optional wax, and a colorant system including a violet pigment such as Pigment Violet 23, Pigment Violet 3, and combinations thereof, present in an amount of from about 1.7 to about 3.8 percent by weight of the toner, in combination with a cyan pigment such as Pigment Blue 61, Pigment Blue 15:3, Pigment Blue 15:4, Pigment Blue 1, Pigment Blue 15:1, Pigment Blue 15:2, and combinations thereof, present in an amount of from about 1.9 to about 4.0 percent by weight of the toner, to form a primary slurry; aggregating the at least one resin and the colorant system with an aggregating agent to form aggregated particles; coalescing the aggregated particles to form toner particles; and recovering the toner particles, wherein the blue toner matches the color of a blue selected from the group consisting of Pantone Blue 072 and Pantone Reflex Blue within a human perception limit ( $\Delta E_{2000}$ ) of less than about 3.

### BRIEF DESCRIPTION OF THE DRAWINGS

Various embodiments of the present disclosure will be described herein below with reference to the figures wherein:

FIG. 1 is a CIELAB  $a^*$ - $b^*$  plot ( $a^*$  corresponds to the red/green value and  $b^*$  denotes the amount of yellow/blue) of Pantone primary colors and CMYK colors available for forming a blue toner;

FIG. 2 is a contour plot of lightness ( $L^*$ ) as a function of loadings of Pigment Violet 23 (PV23) and Pigment Blue 15:3 (PB 15-3) in a toner in accordance with the present disclosure, deposited at 0.45 mg/cm<sup>2</sup>;

FIG. 3 is a contour plot of chroma (C) as a function of loadings of Pigment Violet 23 (PV23) and Pigment Blue 15:3 (PB 15-3) in a toner in accordance with the present disclosure, deposited at 0.45 mg/cm<sup>2</sup>; and

FIG. 4 is a contour plot of hue (h) as a function of loadings of Pigment Violet 23 (PV23) and Pigment Blue 15:3 (PB 15-3) in a toner in accordance with the present disclosure, deposited at 0.45 mg/cm.

It is noted that the drawings of the present disclosure are not to scale. The drawings are intended to depict only typical embodiments of the present disclosure, and therefore should not be considered as limiting the scope of the present disclosure. In the drawings, like numbering represents like elements between the drawings.

#### DETAILED DESCRIPTION

The present disclosure provides toners and systems which may include such toners. In embodiments, a toner of the present disclosure may include a blue toner suitable for use in a color printing system, as an additional colorant besides a cyan, magenta, yellow and/or black.

The present disclosure uses a device independent color space to consistently track a set of target colors. L\*, a\*, b\* are the CIE (Commission Internationale de L'éclairage) color standards utilized in the modeling. L\* defines lightness, a\* corresponds to the red/green value, and b\* denotes the amount of yellow/blue, which corresponds to the way people perceive color. A neutral color is a color where a\*=b\*=0. Resin

Toners of the present disclosure may include any latex resin suitable for use in forming a toner. Such resins, in turn, may be made of any suitable monomer. Suitable monomers useful in forming the resin include, but are not limited to, styrenes, acrylates, methacrylates, butadienes, isoprenes, acrylic acids, methacrylic acids, acrylonitriles, diols, diacids, diamines, diesters, diisocyanates, combinations thereof, and the like. Any monomer employed may be selected depending upon the particular polymer to be utilized.

In embodiments, the resin may be a polymer resin including, for example, resins based on styrene acrylates, styrene butadienes, styrene methacrylates, and more specifically, poly(styrene-alkyl acrylate), poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl acrylate), poly(alkyl methacrylate-aryl acrylate), poly(aryl methacrylate-alkyl acrylate), poly(alkyl methacrylate-acrylic acid), poly(styrene-alkyl acrylate-acrylonitrile-acrylic acid), poly(styrene-1,3-diene-acrylonitrile-acrylic acid), poly(alkyl acrylate-acrylonitrile-acrylic acid), poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene), poly(styrene-propyl acrylate), poly(styrene-butyl acrylate), poly(styrene-butadiene-acrylic acid), polystyrene-butadiene-methacrylic acid), poly(styrene-butadiene-acrylonitrile-acrylic acid), poly(styrene-butyl acrylate-acrylic acid), poly(styrene-butyl acrylate-meth-

acrylic acid), poly(styrene-butyl acrylate-acrylonitrile), poly(styrene-butyl acrylate-acrylonitrile-acrylic acid), poly(styrene-butadiene), poly(styrene-isoprene), polystyrene-butyl methacrylate), poly(styrene-butyl acrylate-acrylic acid), poly(styrene-butyl methacrylate-acrylic acid), poly(butyl methacrylate-butyl acrylate), poly(butyl methacrylate-acrylic acid), poly(acrylonitrile-butyl acrylate-acrylic acid), and combinations thereof. The polymers may be block, random, or alternating copolymers.

10 In other embodiments, the polymer utilized to form the resin may be a polyester resin. Suitable polyester resins include, for example, sulfonated, non-sulfonated, crystalline, amorphous, combinations thereof, and the like. The polyester resins may be linear, branched, combinations thereof, and the like. Polyester resins may include, in embodiments, those resins described in U.S. Pat. Nos. 6,593,049 and 6,756,176, the disclosures of each of which are hereby incorporated by reference in their entirety. Suitable resins may also include a mixture of an amorphous polyester resin and a crystalline 15 polyester resin as described in U.S. Pat. No. 6,830,860, the disclosure of which is hereby incorporated by reference in its entirety.

In embodiments, the resin may be a polyester resin formed by reacting a diol with a diacid or diester in the presence of an optional catalyst. For forming a crystalline polyester, suitable organic diols include aliphatic diols having from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nananediol, 1,10-decanediol, 1,12-dodecanediol, ethylene glycol, combinations thereof, and the like. The aliphatic diol may be, for example, selected in an amount of from about 40 to about 60 mole percent, in embodiments from about 42 to about 55 mole percent, in embodiments from about 45 to about 53 mole percent of the resin.

Examples of organic diacids or diesters selected for the preparation of the crystalline resins include oxalic acid, succinic acid, glutaric acid, adipic acid, suberic acid, azelaic acid, fumaric acid, maleic acid, dodecanedioic acid, sebamic acid, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof, and combinations thereof. The organic diacid may be selected in an amount of, 25 for example, in embodiments from about 40 to about 60 mole percent, in embodiments from about 42 to about 55 mole percent, in embodiments from about 45 to about 53 mole percent.

Examples of crystalline resins include polyesters, polyamides, polyimides, polyolefins, polyethylene, polybutylene, polyisobutylene, ethylenepropylene copolymers, ethylene-vinyl acetate copolymers, polypropylene, mixtures thereof, and the like. Specific crystalline resins may be polyester based, such as polyethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copolypoly(ethylene-adipate), poly(decylene-sebacate), poly(decylene-decanoate), poly(ethylene-decanoate), poly(ethylene-dodecanoate), poly(nonylene-sebacate), poly(nonylene-decanoate), copoly(ethylene-fumarate)-copolypoly(ethylene-sebacate), copoly(ethylene-

fumarate)-copol(ethylene-decanoate), copoly(ethylene-fumarate)-copol(ethylene-dodecanoate), and combinations thereof.

The crystalline resin may be present, for example, in an amount of from about 5 to about 50 percent by weight of the toner components, in embodiments from about 10 to about 35 percent by weight of the toner components. The crystalline resin can possess various melting points of, for example, from about 30° C. to about 120° C., in embodiments from about 50° C. to about 90° C. The crystalline resin may have a number average molecular weight (Mn), as measured by gel permeation chromatography (GPC) of, for example, from about 1,000 to about 50,000, in embodiments from about 2,000 to about 25,000, and a weight average molecular weight (Mw) of, for example, from about 2,000 to about 100,000, in embodiments from about 3,000 to about 80,000, as determined by Gel Permeation Chromatography using polystyrene standards. The molecular weight distribution (Mw/Mn) of the crystalline resin may be, for example, from about 2 to about 6, in embodiments from about 3 to about 4.

Examples of diacid or diesters selected for the preparation of amorphous polyesters include dicarboxylic acids or diesters such as terephthalic acid, phthalic acid, isophthalic acid, fumaric acid, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 55 mole percent of the resin, in embodiments from about 45 to about 53 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanediethanol, 1,3-cyclohexanediethanol, xylenediethanol, cyclohexanediol, diethylene glycol, bis(2-hydroxyethyl)oxide, dipropylene glycol, dibutylene, and combinations thereof. The amount of organic diol selected can vary, and may be present, for example, in an amount from about 40 to about 60 mole percent of the resin, in embodi-

ments from about 42 to about 55 mole percent of the resin, in embodiments from about 45 to about 53 mole percent of the resin.

In embodiments, suitable amorphous resins include polyesters, polyamides, polyimides, polyolefins, polyethylene, polybutylene, polyisobutylene, ethylene-propylene copolymers, ethylene-vinyl acetate copolymers, polypropylene, combinations thereof, and the like. Examples of amorphous resins which may be utilized include alkali sulfonated-polyester resins, branched alkali sulfonated-polyester resins, alkali sulfonated-polyimide resins, and branched alkali sulfonated-polyimide resins. Alkali sulfonated polyester resins may be useful in embodiments, such as the metal or alkali salts of copoly(ethylene-terephthalate)-copol(ethylene-5-sulfo-isophthalate), copoly(propylene-terephthalate)-copol(propylene-5-sulfo-isophthalate), copoly(diethylene-terephthalate)-copol(diethylene-5-sulfo-isophthalate), copoly(propylene-diethylene-terephthalate)-copol(propylene-diethylene-5-sulfoisophthalate), copoly(propylene-butylene-terephthalate)-copol(propylene-butylene-5-sulfo-isophthalate), and copoly(propoxylated bisphenol-A-fumarate)-copol(propoxylated bisphenol A-5-sulfo-isophthalate).

In embodiments, an unsaturated, amorphous polyester resin may be utilized as a latex resin. Examples of such resins include those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butoxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butoxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butoxylated bisphenol co-itaconate), poly(co-propoxylated bisphenol co-ethoxylated bisphenol co-itaconate), poly(1,2-propylene itaconate), and combinations thereof. In embodiments, the amorphous resin utilized in the core may be linear.

In embodiments, a suitable amorphous polyester resin may be a poly(propoxylated bisphenol A co-fumarate) resin having the following formula (I):



ments from about 42 to about 55 mole percent of the resin, in embodiments from about 45 to about 53 mole percent of the resin.

Polycondensation catalysts which may be utilized for either the crystalline or amorphous polyesters include tetraalkyl titanates, dialkyltin oxides such as dibutyltin oxide,

wherein m may be from about 5 to about 1000. Examples of such resins and processes for their production include those disclosed in U.S. Pat. No. 6,063,827, the disclosure of which is hereby incorporated by reference in its entirety.

An example of a linear propoxylated bisphenol A fumarate resin which may be utilized as a latex resin is available under

the trade name SPARII from Resana S/A Industrias Quimicas, Sao Paulo Brazil. Other propoxylated bisphenol A fumarate resins that may be utilized and are commercially available include GTUF and FPESL-2 from Kao Corporation, Japan, and EM181635 from Reichhold, Research Triangle Park, N.C. and the like.

Suitable crystalline resins include those disclosed in U.S. Patent Application Publication No. 2006/0222991, the disclosure of which is hereby incorporated by reference in its entirety. In embodiments, a suitable crystalline resin may be composed of ethylene glycol and a mixture of dodecanedioic acid and fumaric acid co-monomers with the following formula:

(II)



wherein b is from about 5 to about 2000 and d is from about 5 to about 2000.

In embodiments, a suitable crystalline resin utilized in a toner of the present disclosure may have a molecular weight of from about 10,000 to about 100,000, in embodiments from about 15,000 to about 30,000.

One, two, or more resins may be used in forming a toner. In embodiments where two or more resins are used, the resins may be in any suitable ratio (e.g., weight ratio) such as, for instance, from about 1% (first resin)/99% (second resin) to about 99% (first resin)/1% (second resin), in embodiments from about 10% (first resin)/90% (second resin) to about 90% (first resin)/10% (second resin).

As noted above, in embodiments, the resin may be formed by emulsion aggregation methods. Utilizing such methods, the resin may be present in a resin emulsion, which may then be combined with other components and additives to form a toner of the present disclosure.

The polymer resin may be present in an amount of from about 65 to about 95 percent by weight, or preferably from about 75 to about 85 percent by weight of the toner particles (that is, toner particles exclusive of external additives) on a solids basis. The ratio of crystalline resin to amorphous resin can be in the range from about 1:99 to about 30:70, such as from about 5:95 to about 25:75, in some embodiments from about 5:95 to about 15:95.

#### Toner

The resins described above, in embodiments a combination of polyester resins, for example an amorphous resin and a crystalline resin, may be utilized to form toner compositions. Such toner compositions may include optional colorants, waxes, and other additives. Toners may be formed utilizing any method within the purview of those skilled in the art including, but not limited to, emulsion aggregation methods.

#### Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic

surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl 10 cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy)ethanol, available from Rhone-Poulenc as IGEPAL CA-210<sup>TM</sup>, IGEPAL CA-520<sup>TM</sup>, IGEPAL CA-720<sup>TM</sup>, IGEPAL CO-890<sup>TM</sup>, IGEPAL CO-720<sup>TM</sup>, IGEPAL CO-290<sup>TM</sup>, IGEPAL CA-210<sup>TM</sup>, 20 ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecyl naphthalene sulfate, dialkyl benzenealkyl sulfates and sulfonates, acids such as abitic acid available from Aldrich, NEOGEN R<sup>TM</sup>, NEOGEN 30 SCT<sup>TM</sup> obtained from Daiichi Kogyo Seiyaku, combinations thereof, and the like. Other suitable anionic surfactants include, in embodiments, DOWFAX<sup>TM</sup> 2A1, an alkyl diphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually 40 positively charged, include, for example, alkylbenzyl dimethyl ammonium chloride, dialkyl benzenealkyl ammonium chloride, lauryl trimethyl ammonium chloride, alkylbenzyl methyl ammonium chloride, alkylbenzyl dimethyl ammonium bromide, benzalkonium chloride, cetyl pyridinium bromide, C12, C15, C17 trimethyl ammonium bromides, halide salts of quaternized polyoxyethylalkylamines, dodecylbenzyl triethyl ammonium chloride, MIRAPOL<sup>TM</sup> and ALKAQUAT<sup>TM</sup>, available from Alkaril Chemical Company, SANIZOL<sup>TM</sup> (benzalkonium chloride), available from Kao 50 Chemicals, and the like, and mixtures thereof.

#### Colorants

As the colorant to be added, various known suitable colorants, such as dyes, pigments, mixtures of dyes, mixtures of 55 pigments, mixtures of dyes and pigments, and the like, may be included in the toner. The colorant may be included in the toner in an amount of, for example, about 0.1 to about 35 percent by weight of the toner, or from about 1 to about 15 weight percent of the toner, or from about 3 to about 10 percent by weight of the toner.

As examples of suitable colorants, mention may be made 60 of carbon black like REGAL 330<sup>®</sup>; magnetites, such as Mobay magnetites MO8029<sup>TM</sup>, MO8060<sup>TM</sup>; Columbian magnetites; MAPICO BLACK<sup>TM</sup> and surface treated magnetites; Pfizer magnetites CB4799<sup>TM</sup>, CB5300<sup>TM</sup>, CB5600<sup>TM</sup>, 65 MCX6369<sup>TM</sup>; Bayer magnetites, BAYFERROX 8600<sup>TM</sup>, 8610<sup>TM</sup>; Northern Pigments magnetites, NP604<sup>TM</sup>, NP608<sup>TM</sup>; Magnox magnetites TMB-100<sup>TM</sup>, or TMB-104<sup>TM</sup>; and the

like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals, HELIOGEN BLUE L6900<sup>TM</sup>, D6840<sup>TM</sup>, D7080<sup>TM</sup>, D7020<sup>TM</sup>, PYLAM OIL BLUE<sup>TM</sup>, PYLAM OIL YELLOW<sup>TM</sup>, PIGMENT BLUE 1<sup>TM</sup> available from Paul Uhlich & Company, Inc., PIGMENT VIOLET 1<sup>TM</sup>, PIGMENT RED 48<sup>TM</sup>, LEMON CHROME YELLOW DCC 1026<sup>TM</sup>, E.D. TOLUIDINE RED<sup>TM</sup> and BON RED C<sup>TM</sup> available from Dominion Color Corporation, Ltd., Toronto, Ontario, NOVAPERM YELLOW FGL<sup>TM</sup>, HOSTAPERM PINK E<sup>TM</sup> from Hoechst, and CINQUASIA MAGENTA<sup>TM</sup> available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyans include copper tetra(oc-tadecyl sulfonamido) phthalocyanine, x-copper phthalocya-nine pigment listed in the Color Index as CI 74160, CI Pigment Blue, Pigment Blue 15:3, Pigment Blue 15:4, and Anthrathrene Blue, identified in the Color Index as CI 69810, Special Blue X-2137, and the like. Illustrative examples of yellows are diarylide yellow 3,3-dichlorobenzidine acetoac- etanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Per-manent Yellow FGL. Colored magnetites, such as mixtures of MAPICO BLACK<sup>TM</sup>, and cyan components may also be selected as colorants. Other known colorants can be selected, such as Levanyl Black A-SF (Miles, Bayer) and Sunperse Carbon Black LHD 9303 (Sun Chemicals), and colored dyes such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing, and the like.

#### Blue Toner

In embodiments, toners of the present disclosure include blue toners. Blue toners of the present disclosure may include

a colorant system including more than one color. In the present disclosure, a model is provided that can be used to predict the pigment concentrations required to produce a given set of CIELAB values, in embodiments, for a blue toner. Such a model can then be used to derive the exact formulation needed to match the PANTONE<sup>®</sup> blue color standard, PANTONE<sup>®</sup> Blue 072 and/or PANTONE<sup>®</sup> Reflex Blue, or closely related shades of blue.

Color accuracy is generally quantified using the color error factor  $\Delta E_{2000}$ , which converts CIELAB color data ( $L^*$ ,  $a^*$  and  $b^*$ ) for a pair of colors into a single number expressing the "distance" between these colors. The formula for  $\Delta E_{2000}$  uses weighting to compensate for variation in the ability of the human eye to discriminate closely related shades within particular regions of the visible spectrum. When  $\Delta E_{2000} < 3$ , the two colors are generally accepted to be indistinguishable to the human eye.

The PANTONE<sup>®</sup> Matching System of 14 color primaries includes two blue variants that lie between cyan and violet on the color wheel. These colors, PANTONE<sup>®</sup> Blue 072 and PANTONE<sup>®</sup> Reflex Blue, lie within 2.5  $\Delta E_{2000}$  units of one another in the Solid Pantone in the color sample book provided with iGen3<sup>TM</sup> photocopier from Xerox Corporation meaning that they are largely indistinguishable to the naked eye. Upon reviewing FIG. 1, a CIELAB  $a^*$ - $b^*$  plot of PANTONE<sup>®</sup> primary colors and CMYK colors available for a commercially available printer, the DocuColor 8000 printer from Xerox, a toner designed to match one of these primary blue colors should also match the other with a reasonably low  $\Delta E_{2000}$  while providing extended gamut coverage of blue colors for custom-color applications.

Prior to describing the present disclosure in further detail, it will first be helpful to define various terms that will be used throughout the following discussion. For example:

The term "color" may refer to the representation of a vector of values which characterize all or a portion of the image intensity information. It could represent red, green, and blue intensities in an RGB color space or a single luminosity in a Grayscale color space. Alternatively, it could represent alternative information such as CMY, CMYK, PANTONE<sup>®</sup>, x-ray, infrared, and gamma ray intensities from various spectral wavelength bands.

Unless otherwise indicated, all numbers expressing quantities, conditions, and so forth, used in the specification and claims, are to be understood as being modified in all instances by the term "about." In this application, the use of the singular includes the plural unless specifically stated otherwise. In this application, the use of "or" means "and/or" unless stated otherwise. Furthermore, the use of the term "including," as well as other forms, such as "includes" and "included," is not limiting.

The present disclosure describes equations that relate the CIELAB values of a blue toner to its pigment composition. Different relationships exist depending on the nature of the substrate (e.g., smooth vs. rough) and the toner deposition method (e.g., xerographic vs. filtration). These relationships were derived through statistical analysis of color samples made from toners prepared with pigment blends.

The present disclosure further proposes a blue toner formulation matching the color of PANTONE<sup>®</sup> Blue 072 to within a  $\Delta E_{2000}$  of 3, and a blue toner formulation matching the color of PANTONE<sup>®</sup> Reflex Blue to within a  $\Delta E_{2000}$  of about 3, in embodiments just over 3, where the pigments include at least PV23 and PB15:3, and where the PV23 and PB15:3 pigment loadings and print toner mass per unit area (TMA) of the blue are described by a number of equations for at least either  $a^*$ ,  $b^*$ , and  $L^*$ , or  $C$  and  $h$ , or all of  $a^*$ ,  $b^*$ ,  $L^*$ ,

## 11

C, and h. Examples of such equations are described below, where V represents the printed density of PV23 in mg/cm<sup>2</sup>, and B represents the printed density of PB15:3 in mg/cm<sup>2</sup>.

$$L^*=44.6-1425V-662B+21838VB$$

$$\text{Chroma}=75.9+629V-56B+6681VB$$

$$\text{Hue angle}=287.4+876V-383B+17550VB$$

Chroma and hue angle values can be mathematically converted into a\* and b\* values by equations within the purview of those skilled in the art.

In embodiments, for example, the colorant utilized to provide a blue toner may include at least one violet pigment in combination with at least one cyan pigment. Suitable violet pigments for forming the blue toner include, but are not limited to, violet pigments such as Pigment Violet 23 (PV23), Pigment Violet 3 (PV 3), and combinations thereof. The violet pigment may be present in amounts of from about 0.5 percent by weight to about 10 percent by weight of the colorant system, in embodiments from about 1 percent by weight to about 8 percent by weight of the colorant system, in embodiments from about 1.7 percent by weight to about 3.8 percent by weight of the colorant system. The colorant system may also include a cyan pigment. Suitable cyan pigments include Pigment Blue 61 (PB61), Pigment Blue 15:3 (PB 15:3), Pigment Blue 15:4 (PB15:4), Pigment Blue 1, Pigment Blue 15:1, Pigment Blue 15:2, and combinations thereof, in amounts from about 0.1 percent by weight to about 10 percent by weight of the colorant system, in embodiments from about 0.5 percent by weight to about 5 percent by weight of the colorant system, in embodiments from about 1.9 percent by weight to about 4.0 percent by weight of the colorant system.

The colorant system of the present disclosure may be present in a toner in an amount of from about 1 percent by weight to about 15 percent by weight of the toner, in embodiments from about 2 percent by weight to about 8 percent by weight of the toner.

Toners of the present disclosure may be able to obtain a toner mass per area (TMA) of from about 0.2 mg/cm<sup>2</sup> to about 1.5 mg/cm<sup>2</sup>, in embodiments from about 0.3 mg/cm<sup>2</sup> to about 0.7 mg/cm<sup>2</sup>.

A blue toner of the present disclosure may have a lightness (L\*) of from about 19 to about 27, in embodiments from about 20 to about 24.

A blue toner of the present disclosure may have a hue angle of from about 291 degrees to about 299 degrees, in embodiments from about 292 degrees to about 296 degrees.

## Wax

In addition to the polymer binder resin and colorants described above, the toners of the present disclosure also optionally contain a wax, which can be either a single type of wax or a mixture of two or more different waxes. A single wax can be added to toner formulations, for example, to improve particular toner properties, such as toner particle shape, presence and amount of wax on the toner particle surface, charging and/or fusing characteristics, gloss, stripping, offset properties, and the like. Alternatively, a combination of waxes can be added to provide multiple properties to the toner composition.

Where utilized, the wax may be combined with the resin in forming toner particles. When included, the wax may be present in an amount of, for example, from about 1 weight percent to about 25 weight percent of the toner particles, in embodiments from about 5 weight percent to about 20 weight percent of the toner particles.

## 12

Waxes that may be selected include waxes having, for example, a weight average molecular weight of from about 500 to about 20,000, in embodiments from about 1,000 to about 10,000. Waxes that may be used include, for example, 5 polyolefins such as polyethylene, polypropylene, and polybutene waxes such as commercially available from Allied Chemical and Petrolite Corporation, for example POLY-WAX<sup>TM</sup> polyethylene waxes from Baker Petrolite, wax emulsions available from Michaelman, Inc. and the Daniels Products Company, EPOLENE N-15<sup>TM</sup> commercially available from Eastman Chemical Products, Inc., and VISCOL 550-PT<sup>TM</sup>, a low weight average molecular weight polypropylene available from Sanyo Kasei K. K.; plant-based waxes, such as carnauba wax, rice wax, candelilla wax, sumacs wax, and 10 jojoba oil; animal-based waxes, such as beeswax; mineral-based waxes and petroleum-based waxes, such as montan wax, ozokerite, ceresin, paraffin wax, microcrystalline wax, and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9

other materials, which may also be optionally in a dispersion (s) including a surfactant, to the emulsion, which may be a mixture of two or more emulsions containing the resin(s). The pH of the resulting mixture may be adjusted by an acid such as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1 parts per hundred (pph) to about 1 pph, in embodiments from about 0.25 pph to about 0.75 pph, in some embodiments about 0.5 pph. This provides a sufficient amount of agent for aggregation.

The gloss of a toner may be influenced by the amount of retained metal ion, such as  $\text{Al}_3^+$ , in the particle. The amount of retained metal ion may be further adjusted by the addition of EDTA. In embodiments, the amount of retained crosslinker, for example  $\text{Al}_3^+$ , in toner particles of the present disclosure may be from about 0.1 pph to about 1 pph, in embodiments from about 0.25 pph to about 0.8 pph, in embodiments about 0.5 pph.

In order to control aggregation and coalescence of the particles, in embodiments the aggregating agent may be metered into the mixture over time. For example, the agent may be metered into the mixture over a period of from about 5 to about 240 minutes, in embodiments from about 30 to about 200 minutes. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the tempera-

ture to, for example, from about 40° C. to about 100° C., and holding the mixture at this temperature for a time from about 0.5 hours to about 6 hours, in embodiments from about hour 1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition 10 of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments from about 45° C. to about 80° C., which may be below the glass transition temperature of the resin as discussed above.

15 In embodiments, the aggregate particles may be of a size of less than about 3 microns, in embodiments from about 2 microns to about 3 microns, in embodiments from about 2.5 microns to about 2.9 microns.

#### Shell Resin

20 In embodiments, an optional shell may be applied to the formed aggregated toner particles. Any resin described above as suitable for the core resin may be utilized as the shell resin. The shell resin may be applied to the aggregated particles by any method within the purview of those skilled in the art. In 25 embodiments, the shell resin may be in an emulsion including any surfactant described above. The aggregated particles described above may be combined with said emulsion so that the resin forms a shell over the formed aggregates. In embodiments, an amorphous polyester may be utilized to form a shell 30 over the aggregates to form toner particles having a core-shell configuration. In some embodiments, a low molecular weight amorphous resin may be utilized to form a shell over the 35 formed aggregates.

The shell resin may be present in an amount of from about 40 10 percent to about 32 percent by weight of the toner particles, in embodiments from about 24 percent to about 30 percent by weight of the toner particles.

Once the desired final size of the toner particles is achieved, the pH of the mixture may be adjusted with a base to a value 45 of from about 6 to about 10, and in embodiments from about 6.2 to about 7. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above. The base may be added in amounts from about 2 to about 25 50 percent by weight of the mixture, in embodiments from about 4 to about 10 percent by weight of the mixture.

#### Coalescence

Following aggregation to the desired particle size, with the formation of an optional shell as described above, the particles 60 may then be coalesced to the desired final shape, the coalescence being achieved by, for example, heating the mixture to a temperature of from about 55° C. to about 100° C., in embodiments from about 65° C. to about 75° C., in embodiments about 70° C., which may be below the melting point of the crystalline resin to prevent plasticization. Higher or lower temperatures may be used, it being understood that the temperature is a function of the resins used for the binder.

Coalescence may proceed and be accomplished over a period of from about 0.1 to about 9 hours, in embodiments from about 0.5 to about 4 hours.

After coalescence, the mixture may be cooled to room temperature, such as from about 20° C. to about 25° C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

#### Additives

In embodiments, the toner particles may also contain other optional additives, as desired or required. For example, the toner may include any known charge additives in amounts of from about 0.1 to about 10 weight percent, and in embodiments of from about 0.5 to about 7 weight percent of the toner. Examples of such charge additives include alkyl pyridinium halides, bisulfates, the charge control additives of U.S. Pat. Nos. 3,944,493, 4,007,293, 4,079,014, 4,394,430 and 4,560, 635, the disclosures of each of which are hereby incorporated by reference in their entirety, negative charge enhancing additives like aluminum complexes, and the like.

Surface additives can be added to the toner compositions of the present disclosure after washing or drying. Examples of such surface additives include, for example, metal salts, metal salts of fatty acids, colloidal silicas, metal oxides, strontium titanates, mixtures thereof, and the like. Surface additives may be present in an amount of from about 0.1 to about 10 weight percent, and in embodiments of from about 0.5 to about 7 weight percent of the toner. Examples of such additives include those disclosed in U.S. Pat. Nos. 3,590,000, 3,720,617, 3,655,374 and 3,983,045, the disclosures of each of which are hereby incorporated by reference in their entirety. Other additives include zinc stearate and AEROSIL R972® available from Degussa. The coated silicas of U.S. Pat. Nos. 6,190,815 and 6,004,714, the disclosures of each of which are hereby incorporated by reference in their entirety, can also be present in an amount of from about 0.05 to about 5 percent, and in embodiments of from about 0.1 to about 2 percent of the toner, which additives can be added during the aggregation or blended into the formed toner product.

The characteristics of the toner particles may be determined by any suitable technique and apparatus. Volume average particle diameter (D50v), Volume Average Geometric Size Distribution (GSDv), and Number Average Geometric Size Distribution (GSDn), may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3. Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH. Toners of the present disclosure may also possess a parent toner charge per mass ratio (Q/M) of from about -5 µC/g to about -90 µC/g, and a final toner charging after surface additive blending of from -15 µC/g to about -80 µC/g.

Utilizing the methods of the present disclosure, desirable gloss levels may be obtained. Thus, for example, the gloss level of a toner of the present disclosure may have a gloss as measured by Gardner Gloss Units (ggu) of from about 20 ggu

to about 100 ggu, in embodiments from about 50 ggu to about 95 ggu, in embodiments from about 60 ggu to about 90 ggu.

In embodiments, toners of the present disclosure may be utilized as ultra low melt (ULM) toners. In embodiments, the dry toner particles, exclusive of external surface additives, may have the following characteristics:

(1) Volume average diameter (also referred to as "volume average particle diameter") of from about 2.5 to about 20 µm, in embodiments from about 2.75 to about 10 µm, in other embodiments from about 3 to about 7.5 µm.

(2) Number Average Geometric Standard Deviation (GSDn) and/or Volume Average Geometric Standard Deviation (GSDv) of from about 1.18 to about 1.30, in embodiments from about 1.19 to about 1.24.

(3) Circularity of from about 0.9 to about 1 (measured with, for example, a Sysmex FPIA 2100 analyzer), in embodiments from about 0.95 to about 0.985, in other embodiments from about 0.96 to about 0.98.

#### Developers

The toner particles thus formed may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

#### Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidene fluoride, available, for example, as KYNAR 301FTM, and/or polymethylmethacrylate, for example having a weight average molecular weight of about 300,000 to about 350,000, such as commercially available from Soken, may be used. In embodiments, polyvinylidene fluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles,

until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu\text{m}$  in size, in embodiments from about 50 to about 75  $\mu\text{m}$  in size, coated with about 0.5% to about 10% by weight, in embodiments from about 0.7% to about 5% by weight of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

#### Imaging

The toners can be utilized for electrostatographic or electrophotographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengeless development (HSD), and the like. These and similar development systems are within the purview of those skilled in the art.

Imaging processes include, for example, preparing an image with an electrophotographic device including a charging component, an imaging component, a photoconductive component, a developing component, a transfer component, and a fusing component. In embodiments, the development component may include a developer prepared by mixing a carrier with a toner composition described herein. The electrophotographic device may include a high speed printer, a black and white high speed printer, a color printer, and the like.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser member. The fusing member can be of any desired or suitable configuration, such as a drum or roller, a belt or web, a flat surface or platen, or the like. The fusing member can be applied to the image by any desired or suitable method, such as by passing the final recording substrate through a nip formed by the fusing member and a back member, which can be of any desired or effective configuration, such as a drum or roller, a belt or web, a flat surface or platen, or the like. In embodiments, a fuser roll can be used. Fuser roll members are contact fusing devices that are within the purview of those skilled in the art, in which pressure from the roll, optionally with the application of heat, may be used to fuse the toner to the

image-receiving medium. Optionally, a layer of a liquid such as a fuser oil can be applied to the fuser member prior to fusing.

In embodiments, a suitable electrostatographic apparatus 5 for use with a toner of the present disclosure may include a housing defining a chamber for storing a supply of toner therein; an advancing member for advancing the toner on a surface thereof from the chamber of said housing in a first direction toward a latent image; a transfer station for transferring toner to a substrate, in embodiments a flexible substrate, the transfer station including a transfer assist member for providing substantially uniform contact between said print substrate and the image-retentive member; a developer unit possessing toner for developing the latent image; and a 10 fuser member for fusing said toner to said flexible substrate.

Traditionally, color printers have used four housings to 15 generate full-color images based on black plus the standard printing colors cyan, magenta, and yellow. This four-color printing system is able to print a wide range of hues with generally good results. However, in embodiments additional 20 housings may be desirable, including printers possessing five housings, six housings, or more, thus giving it the ability to print an extended range of colors (extended gamut). For example, a six housing system could include orange and blue 25 as priority colors for the additional two housings.

With printer platforms with additional color housings, it 30 may be desirable that the newly introduced colors (i.e., orange and blue) be matched to the equivalent PANTONE® standard primaries (PANTONE® Orange and PANTONE® Blue 072 and/or PANTONE® Reflex Blue) due to the prevalence of the PANTONE® system in the printing and graphic-arts industries.

With respect to the present disclosure, the pigments, or 35 mixtures of pigments selected for each toner are noteworthy, and the combination set, or gamut of toners, such as the cyan toner, the magenta toner, the orange toner, the blue toner, the yellow toner, and the black toner, as it is with these pigments, their sizes, and processes thereof that there is enabled the 40 advantages of the present disclosure illustrated herein and including excellent stable triboelectric characteristics, acceptable stable admix properties, superior color resolution, the capability of obtaining any colors desired, that is a full color gamut, for example thousands of different colors and different developed color images, substantial toner insensitivity 45 to relative humidity, toners that are not substantially adversely affected by environmental changes of temperature, humidity, and the like, the provision of separate unmixed toners, such as black, cyan, magenta, yellow, orange, and blue toners, and mixtures thereof with the advantages illustrated herein, and which toners can be selected for the multicolor 50 development of electrostatic images. The specific selection of colored toners with exceptionally well dispersed pigments enables a large color gamut which assures that thousands of colors can be produced.

55 Also, embodiments of the present disclosure may include an electrophotographic imaging and printing apparatus including, in operative relationship, at least an imaging member component, a charging component, six development components, a transfer component, and a fusing component. In 60 embodiments, the development components include a carrier and six toners, respectively. The six toners may be any combination of colored toners, clear toners, fluorescent toners, and the like. In embodiments, the six toners may include a cyan toner, a magenta toner, a yellow toner, an orange toner, a blue toner, and a black toner. Each of the toners may include, for 65 example, a resin and pigment as illustrated herein. In embodiments, the developer components may be in six sepa-

rated housings, wherein one housing contains the cyan toner, the second housing contains a magenta toner, the third housing contains the yellow toner, the fourth housing contains the black toner, the fifth housing contains the orange toner, and the sixth housing contains the blue toner. As noted above, other colored toners, clear toners, fluorescent toners, combinations thereof, and the like, may be included in the housings.

The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 30° C.

## EXAMPLES

### Example 1

A toner was prepared as follows. A mixture of about 302 parts poly(styrene-co-butyl acrylate) polymer latex (about 42% solids), about 80 parts of a polyethylene wax dispersion (about 32% solids), about 53 parts of a Pigment Blue 15:3 dispersion (about 17% solids), about 35 parts of a Pigment Violet 23 dispersion (about 17.5% solids), and about 680 parts water were combined at room temperature. A mixture of about 4 parts poly(aluminum chloride) and about 36 parts 0.02N HNO<sub>3</sub> were slowly added thereto while homogenizing at about 4,000 revolutions per minute (RPM) with an IKA Turrax T-50 homogenizer. The resulting mixture was stirred and heated slowly to about 55° C. to aggregate the mixture, at which point the particle size (as measured on a Beckman-Coulter Counter) was about 5.5 μm.

About 155 parts of a separate poly(styrene-co-butyl acrylate) polymer latex (about 41% solids) was added to the mixture. When the particle size reached about 6.2 μm, about 5.4 parts of an ethylene diamine tetraacetic acid (EDTA) solution (VERSENE 100) was added thereto, the pH of the mixture was adjusted to about 5.4, and the mixture temperature was increased to about 95° C. When the temperature of the toner mixture reached about 95° C., about 100 ml of 0.1% Cu(NO<sub>3</sub>)<sub>2</sub> solution was added and the mixture was held at about 95° C. for about 3 hours.

After cooling to room temperature, the mixture was filtered and the toner particles were washed with water three times and dried. The resulting particles had about 2.5% Pigment Violet 23 and about 3.7% Pigment Blue 15:3 with a particle size of about 6.1 μm, a Volume Average Geometric Standard Deviation (GSD<sub>V</sub>) of about 1.19, a Number Average Geometric Standard Deviation (GSD<sub>N</sub>) of about 1.24, and a circularity of about 0.96.

### Example 2

Preparation of wet deposition ("wet-dep") color samples. A suspension of the toner from Example 1 was prepared in

water containing a small amount of TRITON-X 100 surfactant. An amount of this suspension, corresponding to about 4.32 mg of toner particles, was passed through a nitrocellulose filter membrane through a cup with an exposed surface area of about 9.62 cm<sup>2</sup>. The retained particles and filter paper were dried at room temperature, then enveloped in Mylar film and passed through a GBC laminator set to a temperature of about 135° C.

Pigment Violet 23 (PV 23) and Pigment Blue 15:3 (PB 15:3) were used in varying amounts to prepare a blue toner of the present disclosure. 6 samples with varying amounts of the two pigments were prepared. The pigment loadings included PV 23 in an amount of from about 2% to about 3.5%, and PB 15:3 in an amount of from about 2.2% to about 3.7%.

Fused samples of the toners were prepared at a deposition of about 0.45 mg/cm<sup>2</sup> toner per mass area (TMA) using the wet-deposition (wet-dep) technique and color values were measured. The dependence of the CIELAB values L\*, a\* and b\* (or L\*, chroma and hue angle) on pigment concentration were calculated. The contents of the toner and the results generated are summarized below in Table 1.

TABLE 1

| Sample # | % PV 23 | % PB 15:3 | L*   | A*   | b*    | C    | h     |
|----------|---------|-----------|------|------|-------|------|-------|
| 1        | 2.00    | 2.20      | 27.4 | 31.7 | -75.0 | 81.5 | 292.9 |
| 2        | 2.00    | 3.70      | 24.3 | 29.7 | -75.9 | 81.5 | 291.4 |
| 4        | 3.50    | 3.70      | 17.1 | 42.2 | -75.4 | 86.5 | 299.3 |
| 5        | 3.40    | 2.35      | 19.6 | 42.1 | -74.8 | 85.8 | 299.4 |
| 6        | 2.77    | 3.00      | 20.3 | 38.5 | -75.5 | 84.7 | 297.0 |

The data thus obtained was processed in the SigmaZone DOE PRO software to provide transfer functions for L\*, chroma and hue angle as a function of pigment loading. The DOE PRO software package is commercially available from SigmaZone, and provides for experimental design, analysis and optimization. The resulting contour plots thus obtained for the samples are presented as FIG. 2 (L\*), FIG. 3 (chroma) and FIG. 4 (hue angle) as a function of Pigment Violet 23 and Pigment Blue 15:3 loadings.

The DOE PRO Multiple Response optimizer was used to predict pigment loadings that would match the hue angle and L\* of Pantone Blue 072 with the highest possible chroma. The toner containing 2.5% PV 23 and 3.7% PB 15:3 from Example 1 was predicted to match Pantone Blue 072 within a ΔE<sub>2000</sub> of 0.4.

The toner was prepared and fused samples were generated at 0.45 mg/cm<sup>2</sup> TMA with the wet-dep technique for color measurement. Table 2 below has the predicted and actual CIELAB values for the toner of Example 1 containing 2.5% Pigment Violet 23 and 3.7% Pigment Blue 15:3. The CIELAB values for PANTONE® Blue 072 and PANTONE® Reflex Blue are provided for reference.

TABLE 2

|                                                    | L*   | a*   | B*    | C    | H     | ΔE <sub>2000</sub> rel. to Blue 072 | ΔE <sub>2000</sub> rel. to Reflex Blue |
|----------------------------------------------------|------|------|-------|------|-------|-------------------------------------|----------------------------------------|
| Prediction for toner with 2.5% PV 23, 3.7% PB 15:3 | 21.6 | 34.2 | -76.0 | 83.3 | 294.2 | 0.40                                | 2.54                                   |
| Toner of Example 1 with 2.5% PV 23, 3.7% PB 15:3   | 22.0 | 33.8 | -75.2 | 82.4 | 294.2 | 0.63                                | 2.70                                   |
| Pantone Blue 072                                   | 21.6 | 34.4 | -77.3 | 84.6 | 294.0 | —                                   | 2.49                                   |
| Pantone Reflex Blue                                | 19.6 | 27.7 | -70.4 | 75.7 | 291.5 | 2.49                                | —                                      |

## 21

As demonstrated in Table 2, the toner of Example 1 with about 2.5% PV 23 and about 3.7% PB 15:3 was an excellent match for PANTONE® Blue 072, providing nearly identical hue angle, identical L\*, and chroma closely matched to the Pantone standard. The  $\Delta E_{2000}$  value for this toner relative to PANTONE® Blue 072 was about 0.63, well within the limit of color differentiation by the human eye ( $\Delta E_{2000}=3$ ). Somewhat surprisingly, this wet-dep color sample also matched PANTONE® Reflex Blue with an acceptable  $\Delta E_{2000}$  of about 2.7.

## Example 3

The toner of Example 1, possessing about 2.5% PV 23 and about 3.7% PB 15:3, was used to prepare about 230 grams of developer at about 12% toner concentration (TC). The developer was conditioned overnight in B-zone, charged up in a TURBULA Type T2C mixer operating at 100 rpm for about 10 minutes and printed in a Xerox WCP3545 machine.

Machine laser diode (LD) power was manually controlled to obtain prints at toner mass per unit area (TMA) levels of 0.7, 0.63, 0.55, 0.45, and 0.39 mg/cm<sup>2</sup>. Ten prints were generated at each TMA level on DCEG paper (coated paper, commercially available from Xerox). The data for prints generated at TMA 0.45 mg/cm<sup>2</sup> (nominal) is summarized below in Table 3, which includes CIELAB values, gloss, and  $\Delta E_{2000}$  for wet-deps and prints of the toner of Example 1, as well as CIELAB values for Pantone Blue 072 and Pantone Reflex Blue.

TABLE 3

|                                 | Gloss | L*   | a*   | b*    | C    | h     | $\Delta E_{2000}$ rel. to PANTONE Blue 072 | $\Delta E_{2000}$ rel. to PANTONE Reflex Blue |
|---------------------------------|-------|------|------|-------|------|-------|--------------------------------------------|-----------------------------------------------|
| Example 1 toner, wet-deps       | —     | 22.0 | 33.8 | -75.2 | 82.4 | 294.2 | 0.63                                       | 2.70                                          |
| Example 1 toner, machine prints | 60.1  | 23.7 | 29.0 | -68.8 | 74.7 | 292.8 | 2.33                                       | 3.25                                          |
| PANTONE ® Blue 072              | —     | 21.6 | 34.4 | -77.3 | 84.6 | 294.0 | —                                          | 2.49                                          |
| PANTONE ® Reflex Blue           | —     | 19.6 | 27.7 | -70.4 | 75.7 | 291.5 | 2.49                                       | —                                             |

As can be seen from the data in Table 3, a slight shift in hue angle and L\* was observed relative to wet-dep values, along with a significant decrease in chroma, as expected from the reduced gloss of an electrophotographic print. However, the CIELAB values of the machine prints relative to PANTONE® Blue 072 indicated that these differences were too minor to be detected by the human eye ( $\Delta E_{2000}=2.33$ ). The color of the machine prints matched PANTONE® Reflex Blue within a  $\Delta E_{2000}$  of 3.25, a difference that would be barely detectable to trained observers.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A blue toner, comprising:  
at least one resin;  
an optional wax; and

## 22

a colorant system comprising a violet pigment selected from the group consisting of Pigment Violet 23, Pigment Violet 3, and combinations thereof, in combination with a cyan pigment selected from the group consisting of Pigment Blue 61, Pigment Blue 15:3, Pigment Blue 15:4, Pigment Blue 1, Pigment Blue 15:1, Pigment Blue 15:2, and combinations thereof,  
wherein the blue toner matches the color of a blue selected from the group consisting of Pantone Blue 072 and Pantone Reflex Blue within a human perception limit ( $\Delta E_{2000}$ ) of less than about 3 in the absence of other pigments.

2. The blue toner of claim 1, wherein the at least one resin comprises styrenes, acrylates, methacrylates, butadienes, isoprenes, acrylic acids, methacrylic acids, acrylonitriles, and combinations thereof.

3. The blue toner of claim 1, wherein the at least one resin comprises a styrene-butyl acrylate resin.

4. The blue toner of claim 1, wherein the at least one resin comprises at least one amorphous polyester resin, optionally in combination with at least one crystalline polyester resin.

5. The blue toner of claim 1, wherein the violet pigment is present in an amount from about 1.7 to about 3.8 percent by weight of the colorant system, and the cyan pigment is present in an amount from about 1.9 to about 4.0 percent by weight of the colorant system.

6. The blue toner of claim 1, wherein the colorant system is present in an amount from about 1 to about 15 percent by

weight of the toner, and wherein the toner has a toner mass per unit area of from about 0.2 mg/cm<sup>2</sup> to about 1.5 mg/cm<sup>2</sup>.

7. The blue toner of claim 1, wherein the wax is present in an amount of from about 1 weight percent to about 25 weight percent of the toner particles.

8. The blue toner according to claim 1, wherein particles comprising the toner are of a size of from about 2.5 microns to about 20 microns.

9. The blue toner according to claim 1, wherein the toner has a lightness (L\*) of from about 19 to about 27, and a hue angle of from about 291 degrees to about 299 degrees.

10. A blue toner, comprising:  
at least one amorphous polyester resin in combination with  
at least one crystalline polyester resin;  
a wax; and

a colorant system comprising a violet pigment selected from the group consisting of Pigment Violet 23, Pigment Violet 3, and combinations thereof, in combination with a cyan pigment selected from the group consisting of Pigment Blue 61, Pigment Blue 15:3, Pigment Blue 15:4, Pigment Blue 1, Pigment Blue 15:1, Pigment Blue 15:2, and combinations thereof,  
wherein the blue toner matches the color of a blue selected from the group consisting of Pantone Blue 072 and Pantone Reflex Blue within a human perception limit ( $\Delta E_{2000}$ ) of less than about 3 in the absence of other pigments.

11. The blue toner of claim 10, wherein the at least one amorphous polyester resin is of the formula:



wherein m may be from about 5 to about 1000, and the optional crystalline polyester resin is of the formula:



wherein b is from about 5 to about 2000 and d is from about 5 to about 2000.

12. The blue toner of claim 10, wherein the violet pigment is present in an amount from about 1.7 to about 3.8 percent by weight of the colorant system, and the cyan pigment is present in an amount of from about 1.9 to about 4.0 percent by weight of the colorant system.

13. The blue toner of claim 10, wherein the colorant system is present in an amount from about 1 to about 15 percent by weight of the toner.

14. The blue toner of claim 10, wherein the toner has a toner mass per unit area of from about 0.2 mg/cm<sup>2</sup> to about 1.5 mg/cm<sup>2</sup>.

15. The blue toner of claim 10, wherein the wax is present in an amount of from about 1 weight percent to about 25 weight percent of the toner particles.

16. The blue toner according to claim 10, wherein particles comprising the toner are of a size of from about 2.5 microns to about 20 microns.

17. The blue toner according to claim 10, wherein the toner has a lightness (L\*) of from about 19 to about 27, and a hue angle of from about 291 degrees to about 299 degrees.

\* \* \* \* \*